# EUROPEAN PATENT APPLICATION

(11) **EP 4 663 846 A1**
(43) Date of publication of application: **17.12.2025**
(21) Application number: 24461585.2
(22) Date of filing: 13.06.2024
(51) Int. Cl.: D06N 7/00

(54) **A BIODEGRADABLE CARPET**

(71) Applicant: Kowary Carpets Sp. z o.o., 58-400 Kamienna Gora (PL)
(72) Inventor: KOMOR, Krzysztof, 58-300 Walbrzych (PL); STAWIARSKI, Tadeusz, 58-400 Kamienna Gora (PL); LENKO, Robert, 58-500 Jelenia Gora (PL)
(74) Representative: Kancelaria Eupatent.pl Sp. z o.o.

(57) **Abstract**

A biodegradable carpet that is fully woven, comprising: a pile yarn being entirely composed of wool yarn; a carpet weft being constructed from natural jute; a carpet warp being composed of biodegradable fibers; and an adhesive layer utilized for pile yarn attachment being biodegradable. The invention also relates to the use of biodegradable carpet as a component of natural fertilizer.

## Description

The invention pertains to a machine-woven carpets or rugs that is fully biodegradable and at the same time has phytoneutrality features.

### BACKGROUND

The present invention concerns a biodegradable carpet, specifically engineered to decompose naturally over time. Carpets, widely used as floor coverings in various settings such as residential, commercial, and industrial environments, are available in a multitude of types, each with unique materials, designs, and manufacturing techniques.

The majority of the market is dominated by carpets produced using tufted technology based on polymers components such as: polypropylene, nylon, polyester or their blends permanently bonded with natural components. Tufted carpets are typically manufactured by inserting pile yarns into a backing material, which is then bonded with another material to ensure durability and stability. This technology has gained popularity due to its cost-effectiveness, versatility in design, and ease of production.

The fundamental disadvantage of today's carpet constructions is the negative impact on the environment.

Traditionally, carpets have been made from a variety of materials, including wool, nylon, polypropylene, and polyester. These materials are chosen for their durability, aesthetic appeal, and comfort. However, products made of permanently bonded various types of polymers and organic fibers are not suitable for segregation or recycling and permanently pollute the environment. This has raised significant environmental concerns, as the disposal of these carpets contributes to landfill waste and pollution on a similar scale to plastic packaging with a worse impact on the environment as waste that cannot be segregated and recycled.

In the European carpet classification system, there are 33 use classes based on the intended use of the carpet, ranging from light domestic use (class 21) to heavy commercial use (class 33). A carpet belonging to use class 32/33 should exhibit high durability and resistance to wear and tear, as it is designed for general or heavy commercial use. This implies that it should be capable of withstanding high levels of foot traffic and heavy furniture.

Despite the diverse range of carpets available in the market, there is an increasing demand for sustainable and environmentally friendly options. This has led to the exploration of biodegradable materials in carpet manufacturing. Biodegradable fabrics, such as those made from plant fibers, can naturally decompose over time, thereby reducing their environmental impact. Additionally, these materials can be repurposed as natural fertilizers or horticultural fabrics once they have decomposed, further enhancing their sustainability.

However, incorporating biodegradable materials in carpet manufacturing presents certain challenges. These materials must be durable enough to endure daily wear and tear, while also being capable of decomposing naturally at the end of their life cycle. Moreover, the manufacturing process must be modified to accommodate these new materials, which may necessitate significant investment and research.

In summary, despite significant advancements in carpet manufacturing, there remains a need for a high-quality, durable, and biodegradable carpet. The present invention aims to fulfil this need by offering a carpet that is not only suitable for heavy commercial use, but also environmentally friendly.

### SUMMARY

The object of the invention is a biodegradable carpet that is fully woven, comprising: a pile yarn being entirely composed of wool yarn; a carpet weft being constructed from natural jute; a carpet warp being composed of biodegradable fibers; and an adhesive layer (104) utilized for pile yarn attachment being biodegradable.

This composition of the biodegradable carpet and its fully woven design ensure optimal durability of the resulting carpet. Moreover, thanks to the use of only fully biodegradable ingredients, after the carpet is used up, it can be disposed of in an ecological way, e.g. by mixing its fragments with compost and thus obtaining natural fertilizer. The biodegradable carpet can serve as a floor covering in domestic and public spaces, and can also be repurposed as a component for natural fertilizers and horticultural fabric or segregated as organic waste, which is not met by the existing carpet structures.

Preferably, the biodegradable carpet according to the invention, having a durability corresponding to the performance class 32/33 of floor coverings as per BS EN 1307:2014.

Preferably, the wool yarn used for the pile yarn is washed. The washing process removes natural dirt and odour of the animal.

Preferably, the wool yarn used for the pile yarn and its construction is stabilized using hot steam. Stabilization of the wool yarn prevents it from untwisting after cut of pile on the loom.

Preferably, the wool yarn used for the pile yarn is non-dyed.

Preferably the biodegradable fibers used for the carpet warp are selected from a group consisting of: viscose, polylactide (PLA) fibers, polyhydroxyalkanoate (PHA) fibers, organic cotton fibers, hemp fibers, and bamboo fibers.

Preferably, the adhesive layer used for the carpet warp comprises an adhesive selected from a group consisting of: natural latex, starch-based adhesive, protein-based adhesive, cellulose-based adhesive and polylactide-based adhesive (PLA).

The invention also relates to use the biodegradable carpet as a component of natural fertilizer.

### BRIEF DESCRIPTION OF THE DRAWINGS

The invention is illustrated in a representative embodiment in the accompanying drawing, wherein:
Fig. 1 shows a first type of biodegradable carpet weave;
Fig. 2 shows a second type of biodegradable carpet weave;
Fig. 3 shows a third type of biodegradable carpet weave.

### DETAILED DESCRIPTION

The invention pertains to a biodegradable carpet that can be produced using standard carpet-making machinery. It is also characterized by its high durability, qualifying it for inclusion in the 32/33 use class of floor coverings as per BS EN 1307:2014.

The biodegradable carpet of the invention comprises a pile yarn 101 made entirely of wool yarn; a carpet weft 102 constructed from natural jute; a carpet warp 103A, 103B composed of biodegradable fibers; and an adhesive layer 104 utilized to secure the pile yarn 101, which is also biodegradable. The use of these specified materials results in the robust biodegradable carpet that decomposes in a compost environment within a period of up to 2 years without the need to use additional chemicals. This provides an environmentally friendly way to dispose of the carpet after it has been used. This is an important advantage due to the increasing restrictions related to environmental protection and the growing problem of storing large amounts of waste that cannot be recycled and is not biodegradable. The biodegradable carpet of the invention can be utilized as a floor covering in both residential and public spaces, as well as a component for natural fertilizers and horticultural fabric, particularly used biodegradable carpet post-dismantling.

The biodegradable carpet according to the invention is fully woven. Unlike conventional methods, the pile yarn 101 is woven into the biodegradable carpet's structure rather than being tufted. This enhances the biodegradable carpet's quality and durability, while also providing greater design flexibility.

Moreover, the biodegradable carpet of the invention can be produced on standard carpet-making looms, a feat not readily achievable with biodegradable materials. For instance, linen, despite its high tensile strength, is unsuitable for use as a warp on a loom due to the excessive hairiness of the fibers. Linen thread, when in friction against the lamellae and threads of the loom, leaves long fibers on them, causing the thread itself to break. The methods of producing carpets using this technology are known to the person skilled in the art and do not require additional discussion. Figs. 1-3 show exemplary carpet weaves that can be used to produce the biodegradable carpet according to the invention.

Preferably, the wool yarn used for the pile yarn 101 is washed (preferably stabilized using hot steam) wool yarn, which has not undergone the dyeing process. This type of wool yarn ensures optimal biodegradability and is suitable for use in standard looms. Moreover, the hot steam infusion process stabilizes the wool yarn and prevents it from untwisting. Wool, as a pile yarn, provides optimal mechanical properties and has a favorable elemental composition, which is a valuable addition to natural fertilizers after the biodegradation of the biodegradable carpet according to the invention.

Natural jute, which is used as weft, was chosen due to its mechanical properties and biodegradability. It allows for optimal durability of the biodegradable carpet and can be used in standard weaving machines.

Preferably, the biodegradable fibers used for the carpet warp 103A, 103B are selected from a group consisting of: viscose, polylactide (PLA) fibers, polyhydroxyalkanoate (PHA) fibers, organic cotton fibers, hemp fibers, bamboo fibers, with a particular preference for viscose. Polylactide fibers (PLA) are produced from lactic acid, a byproduct of corn starch fermentation. They are biodegradable, compostable, and possess properties akin to polyester fibers. Polyhydroxyalkanoate (PHA) fibers are produced by bacteria from sugars and fats. They are biodegradable, compostable, and possess properties akin to polyester fibers. Organic cotton fibers, hemp fibers and bamboo fibers are natural fibers that are biodegradable and compostable. Moreover, they have appropriate mechanical properties which make them suitable for use as the warp 103A, 103B of the biodegradable carpet according to the invention.

Preferably, the adhesive layer 104 utilized in the biodegradable carpet pile yarn 101 comprises an adhesive selected from a group consisting of: natural latex, starch-based adhesive, protein-based adhesive, cellulose-based adhesive and polylactide (PLA)-based adhesive, with a particular preference for natural latex. The starch-based adhesive is fully biodegradable and poses no environmental hazard. The protein-based adhesive is also biodegradable and exhibits significant resistance to moisture. The cellulose-based adhesive is also biodegradable. The polylactide (PLA) based adhesive is biodegradable and increasingly used. PLA-based adhesives are resistant to moisture and temperature, making them an preferably choice for carpeting.

Table 1 presents the physical and chemical parameters of the components of an embodiment of biodegradable carpet according to the invention, while Table 2 provides an example of the percentages and densities of each component.

**Table 1.**

| Selected physicochemical parameters of the components of the invention | | | | |
|---|---|---|---|---|
| Component | Parameter | Value | Parameter | Value |
| Wool yarn | Composition | 100% sheep wool | Tex | 230x3 |
| Jute yarn | Composition | Stem fibers | Tex | 280-413 |
| Viscose thread | Composition | 100% viscose | Tex | 170 |
| | | | Breaking force | 4000 cN |
| Natural Latex | Composition | Water-based compostable adhesive layer | Dry mass | 47% |
| | | | Brookfield viscosity | 80mPa*s |

**Table 2.**

| Component | Approximate percentage of the invention in eg. 7x7 (Corinthian) construction (comb pitch x weaving density) | kg/m2 |
|---|---|---|
| Pile yarn | 51% | 1,023 |
| Warp | 6% | 0,112 |
| Weft | 31% | 0,630 |
| Adhesive layer | 12% | 0,240 |

### Example 1: Utilization of the Biodegradable Carpet as an Additive in Recycled Fertilizer

Recycled fertilizers are products derived from organic or mineral waste, with their composition varying based on the type of starting material. The composition of these recycled fertilizers can be modified and adjusted to achieve desired properties, such as nutrient concentration, pH, texture, and consistency.

The primary component of the biodegradable carpet, as per the invention, is sheep's wool in the form of yarn. Its elemental composition comprises:
- Carbon, constituting approximately 50-55% of the wool's weight.
- Oxygen, constituting approximately 20-25% of the wool's weight.
- Nitrogen, present in proteins, which constitute approximately 15-20% of the wool's weight.
- Sulfur, present in the amino acids cysteine and methionine, which constitute approximately 3% of the wool's weight.
- Potassium, calcium, magnesium, sodium, present in smaller quantities.

Additionally, sheep's wool contains trace amounts of other elements, such as copper, zinc, iron, manganese, chromium, and molybdenum. The elemental content of wool may vary slightly depending on the sheep species, their age, diet, and the conditions under which they were raised.

Shredded biodegradable carpet can serve as an ingredient for organic fertilizers such as compost. Biodegradable carpet that has been used and destined for disposal can be repurposed for this application. Compost is a fertilizer made from organic waste, such as food scraps, grass clippings, leaves, branches, etc. The composition of compost depends on the type of waste and its processing, but it typically contains nitrogen, phosphorus, potassium, and other minerals and microorganisms that promote plant growth.

Recycled composts can have a positive environmental impact as they contribute to waste reduction and reuse. Moreover, recycled composts are often more affordable and readily available than chemical fertilizers, potentially reducing agricultural production costs.

Prior to adding the biodegradable carpet as a fertilizer ingredient, it should be processed using an appropriate shredding machine. The following description, while not an object of intellectual property protection, is a suggested processing method that shortens the biodegradation period.

A shredding machine equipped with a tugger unit and an output feeder for the ground material consists of several components:
1. Initially, fragments of the biodegradable carpet are fed into the machine via an input feeder. The biodegradable carpet then moves to the tugger assembly, where it undergoes intensive grinding.
2. The tugger assembly comprises several rods with blades that rotate around their axis. The blades on the rods grind and shred the biodegradable carpet into smaller pieces. The tugger assemblies can be arranged in different configurations to achieve the desired biodegradable carpet piece size.
3. After shredding, the biodegradable carpet moves to the output feeder, where it is discharged as ground material. The output feeder can be adjusted to different positions to obtain the desired size of the biodegradable carpet pieces.

Fragments of biodegradable carpet prepared in this way can be mixed with compost and serve as natural fertilizer. The possibility of using a biodegradable carpet after its use as a flooring material in a new role as a component of natural fertilizer is a unique, ecological way of its disposal.

### Example 2: Application of the Biodegradable Carpet as Horticultural Fabric

The biodegradable carpet, destined for disposal due to wear and tear, can be repurposed as a horticultural fabric after dismantling. This application allows for the following benefits:
1. Plant protection from pests and diseases - the nonwoven fabric serves as an effective barrier against pests and diseases that could harm plants. It also provides protection against weather conditions such as strong winds or hail.
2. Promotion of plant growth - the nonwoven fabric creates a warm and moist environment that encourages faster plant growth and development.
3. Frost protection - the nonwoven fabric can be used as a shield against low temperatures, protecting plants from frost.
4. Weed control - the nonwoven fabric inhibits the growth of weeds, reducing the need for herbicides.
5. Yield increase - the nonwoven fabric can enhance yields by protecting plants from pests and diseases and controlling weed growth.
6. Soil protection - the nonwoven fabric prevents soil erosion and nutrient loss, contributing to improved soil quality and productivity.

This use of the biodegradable carpet destined for disposal as horticultural fabric is particularly beneficial in the cultivation of plants that are planned for further replanting and where, after the decomposition of the biodegradable carpet, they can be easily dug out of the soil.

## Claims

1. A biodegradable carpet that is fully woven, comprising:
a pile yarn (101) being entirely composed of wool yarn;
a carpet weft (102) being constructed from natural jute;
a carpet warp (103A, 103B) being composed of biodegradable fibers;
an adhesive layer (104) utilized for pile yarn attachment being biodegradable.

2. The biodegradable carpet according to claim 1, having a durability corresponding to the performance class 32/33 of floor coverings as per BS EN 1307:2014.

3. The biodegradable carpet according to any of the preceding claims, wherein the wool yarn used for the pile yarn (101) is washed.

4. The biodegradable carpet according to claim 3, wherein the wool yarn used for the pile yarn (101) is infused with hot steam.

5. The biodegradable carpet according to any of the preceding claims, wherein the wool yarn used for the pile yarn (101) is non-dyed.

6. The biodegradable carpet according to any of the preceding claims, wherein the biodegradable fibers used for the carpet warp (103A, 103B) are selected from a group consisting of: viscose, polylactide (PLA) fibers, polyhydroxyalkanoate (PHA) fibers, organic cotton fibers, hemp fibers, and bamboo fibers.

7. The biodegradable carpet according to any of the preceding claims, wherein the adhesive layer (104) used for the carpet warp (103A, 103B) comprises an adhesive selected from a group consisting of: natural latex, starch-based adhesive, protein-based adhesive, cellulose-based adhesive and polylactide-based adhesive (PLA).

8. The biodegradable carpet according to any of the preceding claims for use as a component of natural fertilizer.
